

## UNITED STATES PATENT OFFICE

GEORGE B. HOGABOOM, OF NEW BRITAIN, CONNECTICUT, AND MYRON B. DIGGIN, OF MATAWAN, NEW JERSEY, ASSIGNEES TO HANSON-VAN WINKLE-MUNNING COMPANY, OF MATAWAN, NEW JERSEY, A CORPORATION OF NEW JERSEY

## CADMIUM PLATING COMPOSITION

No Drawing.

Application filed July 21, 1932. Serial No. 623,818.

The present application is a continuation in part of our prior application Serial No. 554,150, filed July 30, 1931.

This invention relates to an improved composition of electrolyte for use in the electrodeposition of cadmium.

The electrodeposition of cadmium has been successfully employed more particularly with alkaline or cyanide solutions. The character of deposit when employing simple solutions of for example cadmium oxide and sodium cyanide in water is not satisfactory, both on account of poor throwing power and on account of the granular, dull or uneven structure of the deposit, which is unsatisfactory for commercial practice.

An important object of our present invention is to provide an improved composition of electrolyte, either in the form of a mixture or composition of dry chemicals ready to be dissolved, or in the form of an already prepared solution, to enable the electroplater to produce cadmium plating of a fine, uniform, dense structure and of a good bright appearance which will greatly enhance the value of the plating both from a protective standpoint and from the standpoint of attractiveness. On account of the increased throwing power which results from the composition employed in accordance with our invention, the electrolyte is particularly advantageous in the plating of irregular-shaped articles or surfaces.

In an attempt to derive a more comprehensive view of the principle to be employed for obtaining the new character of cadmium deposit, we have made extensive investigation of chemical compounds which could be dissolved or suspended in the electroplating solution and control the character of deposit. Such investigation has led us to recognize the peculiar effect of certain types of organic compounds which, so far as we are aware, have not heretofore been proposed for any such purpose. The compounds which we have identified as being useful for this purpose are the five- and six-membered heterocyclic ring compounds, and particularly those compounds which have a five- or six-membered oxygen-containing heterocyclic ring. Com-

pounds of this class may be relatively simple or comparatively complex in their molecular structure, but our investigations indicate that the presence of the oxygen-containing heterocyclic ring in such compounds has a very important effect on the character of the cadmium deposit when such compounds are to be employed in alkaline plating solutions such as for example those which contain sodium cyanide and a cadmium salt in the presence of another alkali compound, such as caustic soda or sodium carbonate.

As examples of compounds having heterocyclic oxygen-containing rings, which we have found to be useful for our present purposes, we may mention furfural, furfuryl alcohol, tetrahydro furfuryl, furoic acid, and haematein. The first four of these compounds contain five-membered oxyheterocyclic rings and the fifth compound contains a six-membered oxyheterocyclic ring.

In making up the composition for use as an electrolyte, considerable latitude is permissible, but typical examples will be given for the purpose of clearly illustrating the invention. In these examples it may be assumed that the major portion of the composition is made up of 85% sodium cyanide and 15% cadmium oxide. Of this mixture, plus the stated amount of one of the addition agents to be added in accordance with our invention, an aqueous solution can be made in proportions of 120 gms. per L. Sufficient of the addition agent is added either to the mixture to be dissolved in water or to the solution already formed, to represent the following proportions:

Furfural..... 5.8 to 11.2 gms. per L.  
Furfuryl alcohol..... 9.0 to 12.0 c. c. per L.  
Tetrahydro furfuryl..... (11.0), (18.0) or (22.0) c. c. per L.

Furoic acid..... 2.0 to 14.0 gms. per L.  
Haematein..... 0.8 to 12.0 gms. per L.

The addition of furoic acid to the usual cyanide plating solution will produce sodium furoate. This salt may, if desired, be added directly in proper amounts, such as for example, to represent a chemical equivalent of the furoic acid mentioned in the foregoing

example. In the commercial sodium furoate, certain impurities of a resinous or gummy nature are often present. These impurities are definitely beneficial rather than detrimental to the brightening of cadmium plating. It is well known that resins or similar condensation products may be obtained by the interaction of the aldehyde, furfural, and caustic soda in aqueous solution. Such furfural-caustic alkali products are themselves brighteners of cadmium plating deposits, and are included within the scope of our present invention. Furthermore, mixtures of two or more addition agents may be employed. For example, a mixture of sodium furoate and furfural-caustic alkali resin in the proportions of 80% furoate and 20% resin is particularly satisfactory. The mixture may be produced in suitable condition for our purpose, by adding 50 gms. caustic soda in 40% aqueous solution to 122 gms. furfural and 100 c. c. water at the boiling temperature, in a suitable vessel fitted with a reflux condenser. After ten minutes refluxing, the resinate solution thus produced may be mixed with an aqueous solution c. 600 gms. sodium furoate and the mixture evaporated to dryness under vacuum of, say, 22 inches. The product in the form of a dry powder containing sodium furoate and the alkali resin is then ready for use in making up the cadmium plating composition. This addition agent may be used in cadmium plating solutions in the proportions of, for example, 2 to 15 gms. per liter of solution. Somewhat smaller proportions will give a noticeable brightening effect, and larger proportions have been used in some cases. In general, it is believed that the proportions of brightener can be increased as the metal concentration is increased. In solutions having a metal concentration of about 15 to 20 gms. per liter, a proportion of 7 or 8 gms. of this brightener per liter of solution, appears to be about the optimum.

The solutions made up in the manner set forth by way of illustration, may be employed at room temperature at a current density of 10 to 15 amperes per square foot of cathode area. This current density may be varied considerably without loss of the beneficial results, and particularly where agitation of the solution is maintained during operation. In the case of haematein, for example, we have successfully employed 30 amperes per square foot of cathode surface by maintaining agitation during the plating operation.

In accordance with well understood principles, cadmium anodes or insoluble anodes or combinations of the two may be employed.

While the above compounds have been mentioned as examples of addition agents or brighteners containing five- and six-membered oxyheterocyclic rings, we wish to be distinctly understood as not limited to the use

of these particular materials. Some of these compounds, such as for example sodium furoate and furfural caustic alkali resin, (and to a somewhat lesser degree haematein,) are superior to the others in that they produce a more marked brightening effect upon the cadmium, but the brightening effect is produced also by the others, only not to such a marked extent. The presence of the furan ring appears to be important in the effect.

We claim:—

1. A cyanide cadmium plating composition comprising an oxyheterocyclic ring compound.
2. A cyanide cadmium plating composition comprising an oxyheterocyclic ring compound in which the ring is more than four-membered and less than seven-membered.
3. A cyanide cadmium plating composition comprising an oxyheterocyclic compound containing the furan ring.
4. A cyanide cadmium plating composition comprising an alkali metal furoate.
5. A cyanide cadmium plating composition comprising haematein.
6. A cyanide cadmium plating composition comprising furfural.
7. A cyanide cadmium plating composition comprising a caustic alkali furfural resin.
8. A cyanide cadmium plating composition comprising an alkali metal furoate and a caustic alkali furfural resin.
9. A cyanide cadmium plating composition comprising an alkali metal furoate and a caustic alkali furfural resin in the respective proportions of 80% furoate and 20% resin.
10. A cyanide cadmium plating solution comprising as a brightener in the ratio of from two or fifteen grams of 80% alkali metal furoate and 20% caustic alkali furfural resin per liter solution of fifteen to twenty grams per liter metal concentration.

GEORGE B. HOGABOOM.  
MYRON B. DIGGIN.

110

115

120

125

130